# EUROPEAN PATENT SPECIFICATION

(11) **EP 3 168 323 B1**
(45) Date of publication and mention of the grant of the patent: **22.01.2020**
(21) Application number: 15194434.5
(22) Date of filing: 13.11.2015
(51) Int. Cl.: C23C 4/08, C25D 21/14, C23C 24/04, C23C 30/00, F01D 5/28, C23C 18/16, C23C 4/02, C25D 9/04, C25D 13/02, C25D 15/00, C25D 17/00, C23C 4/129, C23C 4/134, C23F 15/00

(54) **POWER PLANT COMPONENT**
KRAFTWERKKOMPONENTE
COMPOSANT DE CENTRALE ÉLECTRIQUE

(43) Date of publication of application: 17.05.2017
(73) Proprietor: General Electric Technology GmbH, 5400 Baden (CH)
(72) Inventor: Bahraini Hasani, Maryam, 5242 Lupfig (CH); Bossmann, Hans-Peter, 79787 Lauchringen (DE)
(74) Representative: Freigutpartners IP Law Firm

(56) References cited:
- EP-A1- 2 388 354
- US-A1- 2006 166 019
- US-A1- 2011 165 433

## Description

### BACKGROUND OF THE INVENTION

The present invention relates to the technology of power plants. It refers to a power plant component according to of claim 1.

### PRIOR ART

Several power plant components such as compressor blade, steam turbine blade and wind blade undergo water droplet erosion, corrosion and fouling. The best way of protection against these damages is protecting blades (or other components) using multi-function composite coatings.

The steel material that is used for compressor blades in gas turbines suffers from water droplet erosion and corrosion pitting induced cracking as well as fouling.

On-line and off-line washings are performed in required intervals in order to improve the performance of the turbine. By applying functional composite coatings on compressor blades, the off-line washing intervals can be extended; less blade erosion occurs during on-line washing and in high fogging systems compressor efficiency is increased.

In addition gas turbines are used in environments, which are highly corrosive for instance in industrial areas or coastlines and therefore undergo a heavy pitting corrosion.

The presence of aerosols and soot in atmosphere causes fouling formation on the blades that worsens the corrosion.

The existing solutions do not address the main three properties of erosion, corrosion and fouling, especially fouling is not addressed or it is very vague. Or the coating considered as anti-fouling is not erosion resistant and therefore anti-fouling property will be lost during operation. Or coating application methods such as sputtering or CVD and PVD are used which are not cost effective or difficult to apply.

Document US 2010/0247321 A1 presents an article including a metallic substrate. The article further includes a sacrificial layer disposed on a surface of the substrate and an anti-fouling layer disposed on the sacrificial layer. The anti-fouling layer includes a metal-polymer composite. An article including an anti-fouling layer having a nitride is also presented.

Document US 2009/0176110 A1 discloses a coating system and process capable of providing erosion and corrosion-resistance to a component, particularly a steel compressor blade of an industrial gas turbine. The coating system includes a metallic sacrificial undercoat on a surface of the component substrate, and a ceramic topcoat deposited by thermal spray on the undercoat. The undercoat contains a metal or metal alloy that is more active in the galvanic series than iron, and electrically contacts the surface of the substrate. The ceramic topcoat consists essentially of a ceramic material chosen from the group consisting of mixtures of alumina and titania, mixtures of chromia and silica, mixtures of chromia and titania, mixtures of chromia, silica, and titania, and mixtures of zirconia, titania, and yttria.

EP 2 374 916 A1 describes a process for providing a protective coating to a metal surface which comprises applying a nickel or tantalum plate layer to the surface and dispersing particles of a hard material such as diamond, alumina, vanadium nitride, tantalum carbide and/or tungsten carbide within the nickel or tantalum plate layer as the plating is occurring.

EP 2 060 328 A2 discloses a method of forming a composite powder coating which comprises depositing multiple layers of a powder coating composition onto a substrate, wherein adjacent layers are formed of a different powder coating composition; and curing the multiple layers of the powder coating composition in a single thermal curing step. The layers can be used to protect power generation equipment from aqueous corrosion, particle erosion, slurry erosion, fretting, and fouling.

US 8,007,246 B2 provides a method of fabricating a component for a gas turbine engine is provided. The method includes applying a bond coat to at least a portion of the component, applying a dense vertically cracked (DVC) thermal barrier coating to at least a portion of the bond coat using a spray mechanism positioned a first distance from the component, and overlying at least a portion of the DVC thermal barrier coating with a soft coat thermal barrier coating using a spray mechanism that is positioned a second distance away from the component, wherein the second distance is greater than the first distance to facilitate adherence of the soft coating thermal barrier coating to the DVC thermal barrier coating.

### SUMMARY OF THE INVENTION

It is an object of the present invention to provide a power plant component with a functional surface with anti-erosion, anti-corrosion and anti-fouling properties.

It is another object of the invention to provide a power plant component with a composite coating system for providing metal and ceramic surfaces with improved water droplet erosion, enhanced corrosion resistance and enhanced anti-fouling properties.

These and other objects are obtained by a power plant component according to Claim 1.

The power plant component according to the invention comprises a substrate the surface of which is coated with a functionally graded coating of a predetermined thickness, with anti-erosion, anti-corrosion and anti-fouling properties.

It is characterized in that said functionally graded coating comprises a corrosion resistant first means, and an erosion resistant and hydrophobic second means, and that said functionally graded coating is a composite coating consisting of a single layer, whereby the concentration of said corrosion resistant first means and the concentration of said erosion resistant and hydrophobic second means vary gradually along the thickness of said composite coating, whereby the concentration of said corrosion resistant first means varies gradually from a high concentration at the inner side of said composite coating to a low concentration at the outer side of said composite coating, and that the concentration of said erosion resistant and hydrophobic second means varies gradually from a low concentration at the inner side of said composite coating to a high concentration at the outer side of said composite coating.

According to an embodiment of the invention said substrate is a metal or composite polymer substrate.

According to the invention said corrosion resistant first means comprises a metal, ceramic, cermet and/or polymer matrix, in which particles are embedded, whereby the concentration of said particles varies gradually from a high concentration at the inner side of said composite coating to a low concentration at the outer side of said composite coating.

Said particles comprise micro or nano metal, ceramic and/or polymer materials, which provide corrosion protection by electronegativity and/or self-healing reaction.

According to a further embodiment of the invention said corrosion resistant first means comprise a Ni matrix with one of Al, Zn, Zr or Mg particles.

According to the invention said erosion resistant and hydrophobic second means comprises a metal, ceramic, cermet and/or polymer matrix, in which hard ceramic, metallic and/or polymer nano or micro materials are included, whereby the concentration of said materials varies gradually from a low concentration at the inner side of said composite coating to a high concentration at the outer side of said composite coating.

According to the invention said erosion resistant and hydrophobic second means comprises ceramic, metallic or intermetallic particles coated with ceramic or polymer material, whereby said ceramic, metallic or intermetallic particles are erosion resistant and said ceramic or polymer coating material is anti-fouling.

Said ceramic, metallic and/or polymer nano or micro particles or fibers may comprise one of SiC, Al₂O₃, SiO₂, WC, BN, MAX phases (e.g. Ti₃SiC₂, Ti₂AlC, Cr₂AlC), carbon nanotubes (CNTs), graphene oxide and hydrophobic particles, especially of PTFE.

The method for manufacturing a power plant component according to the present disclosure is characterized in that the surface of said substrate is activated and prepared with a thin bonding layer and chemical or mechanical treatments.

According to an embodiment of the method said composite coating is applied by spraying process, especially Atmospheric Plasma Spraying (APS), cold spray, High Voltage Oxide Fuel (HVOF) process, or electro and electroless plating and electrophoretic process.

### BRIEF DESCRIPTION OF THE DRAWINGS

The present invention is now to be explained more closely by means of different embodiments and with reference to the attached drawings.
- Fig. 1: shows the surface structure with a graded composite coating of a component according to an embodiment of the invention;
- Fig. 2: shows a diagram of the thickness-dependant concentration of an erosion resistant material within said graded composite coating of Fig. 1; and
- Fig. 3: shows a diagram of the thickness-dependant concentration of a corrosion resistant material within said graded composite coating of Fig. 1.

### DETAILED DESCRIPTION OF DIFFERENT EMBODIMENTS OF THE INVENTION

The present invention is about producing engineered functional coatings and surfaces for power plant components for example gas turbine compressor blades using new materials, design and processing. New functional surfaces are provided with anti-erosion, anti- corrosion and anti-fouling properties.

The present invention presents a composite coating system for providing metal and ceramic surfaces with improved water droplet erosion, enhanced corrosion resistance and enhanced anti-fouling properties.

The coating comprises only one functionally graded layer, where the required properties of corrosion resistance and erosion resistance and hydrophobic properties are varied gradually along the thickness of the layer.

According to Fig. 1-3 the power plant component 10, e.g. a turbine blade, comprises a substrate 11 made of a metal or a composite polymer the surface of which is covered with composite coating 12. Thickness x of the coating begins at coordinate x1 (inner side) and ends at coordinate x2 (outer side). Composite coating 12 contains corrosion resistant first particles (corrosion resistant first means; small circles in Fig. 1) and erosion resistant and hydrophobic second particles/fibers (erosion resistant and hydrophobic second means; larger circles and tildes in Fig. 1) with different profiles of their concentration c. As shown in Fig. 2 the concentration c of the erosion resistant and hydrophobic particles increases from a low concentration c1 at x1 (inner side) to a high concentration c2 at x2 (outer side). On the other hand (see Fig. 3), the concentration c of the corrosion resistant particles decreases from a high concentration c3 at x1 to a low concentration c4 at x2.

Said substrate 11 may be a metal or composite polymer substrate.

Said corrosion resistant first means comprise a metal, ceramic, cermet and/or polymer matrix, in which particles/fibers are embedded, whereby the concentration of said particles varies gradually from a high concentration at the inner side of said composite coating to a low concentration at the outer side of said composite coating.

Said particles/fibers comprise micro or nano metal, ceramic and/or polymer materials, which provide corrosion protection by electronegativity and/or self-healing reaction.

Furthermore, said corrosion resistant first means may comprise a Ni matrix with one of Al, Zn, Zr or Mg particles.

Said erosion resistant and hydrophobic second means comprise a metal, ceramic, cermet and/or polymer matrix, in which hard ceramic, metallic and/or polymer nano or micro materials are included, whereby the concentration of said materials varies gradually from a low concentration at the inner side of said composite coating to a high concentration at the outer side of said composite coating (see Fig. 2), or said erosion resistant and hydrophobic second means may comprise ceramic, metallic or intermetallic particles coated with ceramic or polymer material, whereby said ceramic, metallic or intermetallic particles are erosion resistant and said ceramic or polymer coating material is anti-fouling. Especially, said ceramic, metallic and/or polymer nano or micro particles or fibers may comprise one of SiC, Al₂O₃, SiO₂, WC, BN, MAX phases (e.g. Ti₃SiC₂, Ti₂AlC, Cr₂AlC), carbon nanotubes (CNTs), graphene oxide and hydrophobic particles, especially of PTFE.

### LIST OF REFERENCE NUMERALS

- 10: power plant component
- 11: substrate
- 12: composite coating
- c,c1,c2,c3,c4: concentration
- x,x1,x2: coating thickness (coordinate)

## Claims

1. Power plant component (10), comprising a substrate (11) the surface of which is coated with a functionally graded coating (12) of a predetermined thickness, with anti-erosion, anti-corrosion and anti-fouling properties, wherein said functionally graded coating (12) comprises a corrosion resistant first means, and an erosion resistant and hydrophobic second means, and that said functionally graded coating is a composite coating (12) consisting of a single layer, whereby the concentration of said corrosion resistant first means and the concentration of said erosion resistant and hydrophobic second means vary gradually along the thickness (x) of said composite coating (12), whereby the concentration of said corrosion resistant first means varies gradually from a high concentration (c3) at the inner side (x1) of said composite coating (12) to a low concentration (c4) at the outer side (x2) of said composite coating (12), and that the concentration of said erosion resistant and hydrophobic second means varies gradually from a low concentration (c1) at the inner side (x1) of said composite coating (12) to a high concentration (c2) at the outer side (x2) of said composite coating (12),
wherein said corrosion resistant first means comprises a metal, ceramic, cermet and/or polymer matrix, in which particles are embedded, whereby the concentration of said particles varies gradually from a high concentration at the inner side of said composite coating to a low concentration at the outer side of said composite coating, and said particles comprise micro or nano metal, ceramic and/or polymer materials, which provide corrosion protection by electronegativity and/or self-healing reaction, and
wherein said erosion resistant and hydrophobic second means comprises:
- a metal, ceramic, cermet and/or polymer matrix, in which hard ceramic, metallic and/or polymer nano or micro materials are included, whereby the concentration of said materials varies gradually from a low concentration at the inner side of said composite coating to a high concentration at the outer side of said composite coating, or
- ceramic, metallic or intermetallic particles coated with ceramic or polymer material, whereby said ceramic, metallic or intermetallic particles are erosion resistant and said ceramic or polymer coating material is anti-fouling.

2. Power plant component as claimed in Claim 1, **characterized in that** said substrate (11) is a metal or composite polymer substrate.

3. Power plant component as claimed in Claim 1, **characterized in that** said corrosion resistant first means comprise a Ni matrix with one of Al, Zn, Zr or Mg particles.

4. Power plant component as claimed in Claim 1, **characterized in that** said ceramic, metallic and/or polymer nano or micro particles or fibers comprises one of SiC, Al₂O₃, SiO₂, WC, BN, MAX phases (e.g. Ti₃SiC₂, Ti₂AlC, Cr₂AlC), carbon nanotubes (CNTs), graphene oxide and hydrophobic particles, especially of PTFE.

## Patentansprüche

1. Kraftwerkkomponente (10), umfassend ein Substrat (11) dessen Oberfläche mit einer funktionellen abgestuften Beschichtung (12) einer vorbestimmten Dicke mit Erosionsschutz-, Korrosionsschutz- und Bewuchsschutzeigenschaften beschichtet ist, wobei die funktionelle abgestufte Beschichtung (12) ein korrosionsbeständiges erstes Mittel und ein erosionsbeständiges und hydrophobes zweites Mittel umfasst, und dass die funktionelle abgestufte Beschichtung eine Verbundbeschichtung (12) ist, die aus einer einzelnen Schicht besteht, wobei die Konzentration des korrosionsbeständigen ersten Mittels und die Konzentration des erosionsbeständigen und hydrophoben zweiten Mittels graduell entlang der Dicke (x) der Verbundbeschichtung (12) variieren, wobei die Konzentration des korrosionsbeständigen ersten Mittels graduell von einer hohen Konzentration (c3) an der inneren Seite (x1) der Verbundbeschichtung (12) zu einer geringen Konzentration (c4) an der äußeren Seite (x2) der Verbundbeschichtung (12) variiert, und dass die Konzentration des erosionsbeständigen und hydrophoben zweiten Mittels graduell von einer geringen Konzentration (c1) an der inneren Seite (x1) der Verbundbeschichtung (12) zu einer hohen Konzentration (c2) an der äußeren Seite (x2) der Verbundbeschichtung (12) variiert,
wobei das korrosionsbeständige erste Mittel ein Metall, Keramik, Cermet und/oder eine Polymermatrix umfasst, in der Partikel eingebettet sind, wobei die Konzentration der Partikel graduell von einer hohen Konzentration an der inneren Seite der Verbundbeschichtung zu einer geringen Konzentration an der äußeren Seite der Verbundbeschichtung variiert, und die Partikel Mikro- oder Nanometall, Keramik und/oder Polymermaterialien umfassen, die einen Korrosionsschutz durch Elektronegativität und/oder selbstheilende Reaktion bereitstellen, und
wobei das erosionsbeständige und hydrophobe zweite Mittel umfasst:
- ein Metall, Keramik, Cermet und/oder eine Polymermatrix in der harte keramische, metallische und/oder polymerische Nano- oder Mikromaterialien enthalten sind, wobei die Konzentration der Materialien graduell von einer geringen Konzentration an der inneren Seite der Verbundbeschichtung zu einer hohen Konzentration an der äußeren Seite der Verbundbeschichtung variiert, oder
- keramische, metallische oder intermetallische Partikel, die mit Keramik- oder Polymermaterial beschichtet sind, wobei die keramischen, metallischen oder intermetallischen Partikel erosionsbeständig sind und das Keramik- oder Polymerbeschichtungmaterial bewuchsschützend ist.

2. Kraftwerkkomponente nach Anspruch 1, **dadurch gekennzeichnet, dass** das Substrat (11) ein Metall- oder Verbundpolymersubstrat ist.

3. Kraftwerkkomponente nach Anspruch 1, **dadurch gekennzeichnet, dass** das korrosionsbeständige erste Mittel eine Ni-Matrix mit einem von Al-, Zn-, Zr- oder Mg-Partikeln umfasst.

4. Kraftwerkkomponente nach Anspruch 1, **dadurch gekennzeichnet, dass** die keramischen, metallischen und/oder polymerischen Nano- oder Mikropartikel oder - fasern eines von SiC, Al₂O₃, SiO₂, WC, BN, MAX-Phasen (z.B. Ti₃SiC₂, Ti₂AlC, Cr₂AlC), Kohlenstoffnanoröhrchen (CNTs), Graphitoxid und hydrophoben Partikeln umfassen, insbesondere aus PTFE.

## Revendications

1. Composant de centrale électrique (10), comprenant un substrat (11) dont la surface est revêtue avec un revêtement à gradient de fonctionnalité (12) ayant une épaisseur prédéterminée, présentant des propriétés anti-érosion, anticorrosion et anti-encrassement, dans lequel ledit revêtement à gradient de fonctionnalité (12) comprend un premier moyen résistant à la corrosion, et un second moyen hydrophobe et résistant à l'érosion, et que ledit revêtement à gradient de fonctionnalité est un revêtement composite (12) consistant en une monocouche, selon lequel la concentration dudit premier moyen résistant à la corrosion et la concentration dudit second moyenne hydrophobe et résistant à l'érosion varient graduellement le long de l'épaisseur (x) dudit revêtement composite (12), selon lequel la concentration dudit premier moyen résistant à la corrosion varie graduellement d'une concentration élevée (c3) au niveau du côté interne (x1) dudit revêtement composite (12) à une concentration basse (c4) au niveau du côté externe (x2) dudit revêtement composite (12), et que la concentration dudit second moyen hydrophobe et résistant à l'érosion varie graduellement d'une concentration basse (c1) au niveau du côté interne (x1) dudit revêtement composite (12) à une concentration élevée (c2) au niveau du côté externe (x2) dudit revêtement composite (12),
dans lequel ledit premier moyen résistant à la corrosion comprend une matrice métallique, céramique, en cermet et/ou polymère, dans laquelle des particules sont incrustées, selon lequel la concentration desdites particules varie graduellement d'une concentration élevée au niveau du côté interne dudit revêtement composite à une concentration basse au niveau du côté externe dudit revêtement composite, et lesdites particules comprennent des micro- ou nano-matériaux métalliques, céramiques et/ou polymères, qui fournissent une protection contre la corrosion par électronégativité et/ou réaction d'auto-réparation, et
dans lequel ledit second moyen hydrophobe et résistant à l'érosion comprend :
- une matrice métallique, céramique, en cermet et/ou polymère, dans laquelle des nano- ou micro-matériaux céramiques, métalliques et/ou polymères durs sont inclus, selon lequel la concentration desdits matériaux varie graduellement d'une concentration basse au niveau du côté interne dudit revêtement composite à une concentration élevée au niveau du côté externe dudit revêtement composite, ou
- des particules céramiques, métalliques ou intermétalliques revêtues avec un matériau céramique ou polymère, selon lequel lesdites particules céramiques, métalliques ou intermétalliques sont résistantes à l'érosion et ledit matériau de revêtement céramique ou polymère est anti-encrassement.

2. Composant de centrale électrique selon la revendication 1, **caractérisé en ce que** ledit substrat (11) est un substrat métallique ou polymère composite.

3. Composant de centrale électrique selon la revendication 1, **caractérisé en ce que** ledit premier moyen résistant à la corrosion comprend une matrice de Ni avec l'une de particules d'Al, Zn, Zr ou Mg.

4. Composant de centrale électrique selon la revendication 1, **caractérisé en ce que** lesdites nano- ou micro-particules ou fibres céramiques, métalliques et/ou polymères comprennent l'un parmi SiC, Al₂O₃, SiO₂, WC, BN, des phases MAX (par exemple Ti₃SiC₂, Ti₂AlC, Cr₂AlC), des nanotubes de carbone (CNT), un oxyde de graphène et des particules hydrophobes, en particulier de PTFE.
